

## UNITED STATES PATENT OFFICE

2,132,902

## FLOTATION PROCESS

Samuel Lenher, Wilmington, Del., assignor to E. I. du Pont de Nemours & Company, Wilmington, Del., a corporation of Delaware

No Drawing. Application June 14, 1934,  
Serial No. 730,551

26 Claims. (Cl. 209—166)

This invention relates to a process for concentrating minerals, and more particularly refers to a froth flotation process whereby a high concentration of minerals which formerly could be obtained only with extreme difficulty are separated in a rapid and extremely efficient manner. Heretofore ores have been subjected to froth flotation processes utilizing a soap or analogous surface active reagents. These reagents were frequently quite inefficient and resulted in the production of a low yield of inferior concentrates. Because of the inefficiency of such processes the froth flotation of many ores was considered impossible, the reason why the aforesaid processes would float some ores and not others being unknown up to the present time, although several theories had been advanced therefor. The aforesaid flotation agents were, furthermore, unsatisfactory in that large quantities thereof were necessary and the conditions of operation had to be maintained within relatively narrow limits.

It is an object of the present invention to avoid the previously-described difficulties and the numerous disadvantages which directly or indirectly resulted therefrom. A further object is to utilize as flotation agents compounds which heretofore were not known to have flotation properties or to be of any value in flotation processes. A still further object is to devise a froth flotation process wherein ores and minerals which formerly could not be concentrated by flotation processes or which were concentrated thereby only with great difficulty may be readily and efficiently separated. A still further object is to explain the reason why prior art flotation agents were unsatisfactory for the flotation of numerous ores, and to instruct one in the means of avoiding such difficulties. Additional objects will be come apparent from a consideration of the following specification and claims.

These objects are attained according to the process of the present invention wherein ores and minerals in general may be concentrated by means of a froth flotation process utilizing compounds containing a positively charged surface active ion. In a more limited sense the invention relates to the froth flotation of non-sulfide ores by means of a compound containing a positively charged surface active ion one of the components of which is a hydrocarbon radical having at least eight carbon atoms. The preferred embodiment of this invention comprises the froth flotation of negatively charged non-sulfide minerals by means of quaternary ammonium com-

pounds containing in the positively charged surface active portion thereof an aliphatic hydrocarbon radical having from twelve to eighteen carbon atoms.

The invention may be more readily understood by a consideration of the following illustrative examples:

*Example 1*

1000 grams of North Carolina feldspar were suspended in water in a Denver Equipment Company flotation cell. To this suspension was added 0.2 gram of cetyl pyridinium bromide dissolved in water. The resulting suspension was agitated and air passed therethrough, the pH value of the circuit being maintained at about 7.0. The ore was immediately and strongly flocculated. A concentrate was obtained consisting of 706 grams of high quality minerals, the tails amounting to 291 grams.

*Example 2*

The preceding example was repeated substituting 0.2 gram of cetyl trimethyl ammonium chloride for the cetyl pyridinium bromide. Upon agitation the ore was immediately and strongly flocculated. A concentrate was obtained weighing 856 grams, the tails amounting to 144 grams.

*Example 3*

Example 1 was again repeated substituting 1000 grams of Manavala Kurichi ilmenite for the feldspar. This ore assayed 90% ilmenite, 7% garnet and 3% miscellaneous minerals. As a flotation agent 0.4 gram of cetyl pyridinium bromide was used. The concentrate weighed 651 grams, and the tails 349 grams.

The preceding examples were repeated substituting a well known flotation agent, namely soap, for the flotation agents used therein. In each case an exceedingly poor yield of low quality concentrate was obtained. The use of soap in the flotation of these ores was, therefore, impracticable.

It is to be understood that in place of the ores floated in the aforementioned examples numerous other sulfide or non-sulfide ores might be substituted. In particular the flotation of ores which are negatively charged was found to be exceedingly satisfactory. The determination of the electrical charge of ore particles is readily made by well known methods of electrophoresis, such as are described in Holmes, Laboratory Manual of Colloid Chemistry, John Wiley & Sons, New York city, second edition, 1928, p. 48; and by Ettisch & Deutsch, Physik. Z. 28, 153 (1927). A

few representative ores coming within this category and floated according to the present instructions with surprisingly good results are the feldspars as a class; quartz; ilmenite; the pyroxenes, 5 the spinels such as picotite and magnetite; the micas such as biotite and muscovite.

While the invention is particularly adapted for the flotation of negatively charged ores it is to be understood that it is not limited thereto 10 and may frequently be used to float positively charged ores. It may be applied to both sulfide and non-sulfide ores. When applied to the former it is in general advisable that the flotation agents described herein be utilized in admixture 15 with the customary flotation agent for sulfide ores. Sulfide flotation agents which may be used in admixture herewith are, for example, xanthates, mercaptans, thioureas, carbamates, etc. In the case of non-sulfide ores the flotation 20 agents described herein may customarily be used without admixing therewith additional flotation agents. However, where the non-sulfide ore to be floated contains a positive charge it is usually advantageous to mix the herein-described flotation agents with soap, soap-like products, water-soluble sulfuric esters of higher normal primary 25 alcohols, sulfonated derivatives of higher fatty acids and higher fatty alcohols, and other flotation agents. The presence of the agents forming the subject matter of the present invention in admixture with other flotation agents results in a more highly selective froth flotation operation, with the consequent production of a higher yield 30 of better quality concentrate than could ordinarily be obtained. The proportion of the individual components in such admixture may vary within wide limits, the agent or agents described herein being used in amounts varying from mere traces to major fractions thereof.

40 The flotation agents comprised herein are broadly compounds containing a positively charged surface active ion. One familiar with the art in view of the present instructions would have no difficulty in determining the compounds 45 which satisfy these requirements. Among the compounds which come within the aforesaid category a class which has been found to possess particular value is the quaternary ammonium compounds. These compounds are especially 50 advantageous when the positively charged ion thereof contains a hydrocarbon radical having at least eight and preferably from twelve to eighteen carbon atoms.

55 In this connection, an aliphatic hydrocarbon radical has been found to be especially advantageous. The negatively charged ion of said compound should preferably possess little or no surface activity, although as long as the surface activity of the positively charged ion is appreciably greater than that of the negatively charged ion the compound will function satisfactorily. Halogen atoms have been found to be particularly suited for use as the negatively charged ion. These atoms possess negligible surface activity and consequently permit the positively charged ion to function with maximum 60 selectivity.

65 In addition to the previously mentioned hydrocarbon radical, the positively charged portion of the flotation agent may advisably contain one or more of the commonly known substituents. For example, aliphatic and/or aromatic radicals which may be further substituted by alkyl, alkoxy, nitro, amino, halogen, carboxy, 70 sulfonic acid, benzoylamino, diphenylamine, etc.

groups. The compound may contain more than one hydrocarbon group of high molecular weight and such group or groups may be further substituted as in the case of the remaining portion of the molecule. Compounds which illustrate such instructions but are not intended as a limitation thereon are:

|                                                                                                                                                          |    |
|----------------------------------------------------------------------------------------------------------------------------------------------------------|----|
| Cetyl trimethyl ammonium bromide or chloride                                                                                                             | 10 |
| Lauryl trimethyl ammonium chloride or iodide                                                                                                             |    |
| Cetyl pyridinium bromide                                                                                                                                 |    |
| Dimethyl benzyl phenyl ammonium chloride sul-<br>fonated in benzyl ring                                                                                  |    |
| Beta diethyl amino ethyl oleyl amide acetate                                                                                                             | 15 |
| Beta diethyl amino ethyl oleyl amide hydrochlo-<br>ride                                                                                                  |    |
| Trimethyl ammonium methyl sulfate or amino<br>oleyl ethylene diamine                                                                                     |    |
| Quaternary ammonium compounds containing at<br>least one aliphatic chain with at least eight<br>and not more than twenty carbon atoms in<br>the molecule | 20 |
| Water-soluble or acid solution soluble compounds<br>of amino cellulose such as chitosan acetate                                                          |    |
| Trimethyl octadecyl ammonium bromide                                                                                                                     | 25 |
| Trimethyl eicosyl ammonium iodide                                                                                                                        |    |
| Octadecyl pyridinium bromide                                                                                                                             |    |
| Trimethyl octadecyl ammonium chloride                                                                                                                    |    |
| Trimethyl dodecyl ammonium bromide                                                                                                                       |    |
| Trimethyl dodecyl ammonium iodide                                                                                                                        | 30 |
| Octadecyl beta hydroxyethyl morpholinium bro-<br>mide                                                                                                    |    |
| Cetyl beta hydroxyethyl morpholinium bromide                                                                                                             |    |
| Triethyl octadecyl ammonium bromide                                                                                                                      |    |
| Triethyl cetyl ammonium bromide                                                                                                                          | 35 |
| Beta stearamidophenyl trimethylammonium<br>methyl sulfate                                                                                                |    |
| Octadecyl pyridinium chloride                                                                                                                            |    |
| Octadecyl pyridinium iodide                                                                                                                              |    |
| Octadecyl alpha picolinium bromide                                                                                                                       | 40 |
| Octadecyl quolininium bromide                                                                                                                            |    |
| Dodecyl pyridinium bromide                                                                                                                               |    |
| Heptadecylamine hydrochloride                                                                                                                            |    |
| Hexadecylamine hydrochloride                                                                                                                             |    |
| Dodecylamine hydrochloride.                                                                                                                              | 45 |

In the past many ores were floated only with great difficulty or were found to be impossible to float because it was never before appreciated that the compounds selected for flotation should be chosen in accordance with the electrical charge 50 present on the ore. For instance, soap was a customary flotation agent for all non-sulfide ores. The surface active portion of soap contains a negative charge. Consequently, where the ore to be floated also contained a negative charge soap 55 was quite inefficient as a flotation agent. The present invention discloses a means of overcoming this difficulty, and permits the particular characteristic of the ore which defeated its flotation in the past to be used to advantage. 60

The flotation agents described herein for the first time, while being particularly adapted to the flotation of negatively charged ore are, as previously mentioned, not restricted thereto. These compounds have in addition to their positive 65 charge an extremely high surface activity. As a result thereof, even when the ore to be floated is positively charged this surface activity of the flotation agent will produce a satisfactory yield of good quality concentrate. The agents described herein contain positively charged particles, ions or micelles. As a result of this phenomenon the surface active particles speedily form agglomerates or flocks on the surface of the ore to be floated and aid to a surprising extent in 70 75

raising said ore to the surface. In addition to bringing the desired ore to the surface the present invention may be so modified that the desired mineral remains submerged and the undesired components of the ore are brought to the surface and separated therefrom.

The present invention permits the use of an exceedingly large number of compounds in the froth flotation of ore. These compounds were heretofore unknown to have flotation properties. As a result of this invention ores which formerly could not be subjected to froth flotation or when so subjected were quite unsatisfactory may now be treated by froth flotation processes with surprisingly good results. The operation is speedy and need not be maintained within narrow limits.

As many apparently widely different embodiments of this invention may be made without departing from the spirit and scope thereof, it is to be understood that the invention is not limited to the specific embodiments thereof except as defined in the appended claims.

I claim:

1. A process for the froth flotation of negatively charged non-sulfide ores which comprises frothing an aqueous suspension of said ores in the presence of an organic compound, the surface active portion of which is a positive ion.

2. The process of claim 1 wherein the positively charged surface active ion contains a hydrocarbon radical having at least eight carbon atoms.

3. A process for the froth flotation of negatively charged minerals which comprises agitating a liquid suspension of said minerals in the presence of a compound containing a positively charged surface active ion, said ion containing an aliphatic hydrocarbon radical having from eight to eighteen carbon atoms.

4. A process for the froth flotation of negatively charged minerals which comprises agitating an aqueous suspension of ore containing said minerals in the presence of a quaternary ammonium compound having a positively charged surface active ion.

45 5. A process for the froth flotation of negatively charged minerals which comprises agitating an aqueous suspension of ore containing said minerals in the presence of an ammonium compound having the following general formula:



wherein R represents an aliphatic hydrocarbon radical having from 8 to 18 carbon atoms, R<sub>2</sub> represents hydrogen or hydrocarbon radicals or both hydrogen and hydrocarbon radicals, having a total valence of 3, and X represents a negatively charged group possessing negligible surface active properties when in solution.

60 6. The process of claim 5 wherein X represents a halogen atom.

7. The process of claim 5 wherein X represents a chlorine, bromine or iodine atom.

65 8. A process for the froth flotation of negatively charged non-sulfide ores which comprises agitating and aerating an aqueous suspension of said ore in the presence of a nitrogen-containing organic flotation agent, the surface active portion of which is positively charged.

70 9. A process for the froth flotation of negatively charged non-sulfide ores which comprises agitating and aerating an aqueous suspension of said ore in the presence of a nitrogen-containing organic compound having a hydrocarbon radical

of at least 8 carbon atoms, the surface active portion of which is positively charged.

10. A process for the froth flotation of negatively charged ores which comprises agitating and aerating an aqueous suspension of said ores in the presence of an ammonium compound having the following general formula:



wherein R represents an aliphatic hydrocarbon radical having from 8 to 18 carbon atoms, R<sub>2</sub> represents hydrogen or hydrocarbon radicals or both hydrogen and hydrocarbon radicals, having a total valence of 3, and X represents chlorine or bromine.

11. A process for the froth flotation of negatively charged ores which comprises agitating and aerating an aqueous suspension of said ores in the presence of an ammonium compound having the general formula:



wherein R<sub>1</sub> represents an aliphatic hydrocarbon radical having from 8 to 18 carbon atoms, R<sub>2</sub>, R<sub>3</sub> and R<sub>4</sub> represent hydrogen atoms, and X represents a halogen atom.

12. A process as set forth in claim 11 wherein the ore treated is quartz.

13. A process for the froth flotation of negatively charged ores which comprises agitating and aerating an aqueous suspension of said ores in the presence of dodecylamine hydrochloride.

14. A process as set forth in claim 13 wherein the ore treated is quartz.

15. A process for the froth flotation of negatively charged ores which comprises agitating and aerating an aqueous suspension of said ores in the presence of an ammonium compound having the following general formula:



wherein R<sub>1</sub> represents an aliphatic hydrocarbon radical having from twelve to eighteen carbon atoms, R<sub>2</sub>, R<sub>3</sub> and R<sub>4</sub> represent hydrogen atoms, and X represents chlorine.

16. A process for the froth flotation of negatively charged ores which comprises agitating and aerating an aqueous suspension of said ores in the presence of a quaternary ammonium compound having the following general formula:



wherein R<sub>1</sub> represents an aliphatic hydrocarbon radical having from 8 to 18 carbon atoms, R<sub>2</sub>, R<sub>3</sub> and R<sub>4</sub> represent hydrocarbon groups, and X represents a halogen atom.

17. A process as set forth in claim 16 wherein the ore treated is a mica.

18. A process for the froth flotation of negatively charged ores which comprises agitating and aerating an aqueous suspension of said ores in the presence of cetyl trimethyl ammonium bromide.

19. A process as set forth in claim 18 wherein the ore treated is muscovite.

20. A process for the froth flotation of negatively charged ores which comprises agitating and aerating an aqueous suspension of said ores

in the presence of a quaternary ammonium compound having the following general formula:

5



wherein  $R_1$  represents an aliphatic hydrocarbon radical having from twelve to eighteen carbon atoms,  $R_2$ ,  $R_3$  and  $R_4$  represent hydrocarbon groups, and  $X$  represents bromine.

10 21. A process for the froth flotation of negatively charged minerals which comprises agitating an aqueous suspension of ore containing said minerals in the presence of a quaternary ammonium compound containing a positively charged surface active ion, said ion containing a hydrocarbon radical having at least 8 carbon atoms.

20 22. A process for the froth flotation of negatively charged ores which comprises agitating and aerating an aqueous suspension of said ores in the presence of a quaternary ammonium compound having the following general formula:

25



wherein  $R_1$  represents an aliphatic hydrocarbon radical having from 8 to 18 carbon atoms, and  $X$  represents a halogen atom.

23. A process as set forth in claim 22 wherein the ore treated is a feldspar. 5

24. A process for the froth flotation of negatively charged ores which comprises agitating and aerating an aqueous suspension of said ores in the presence of cetyl pyridinium bromide.

25. A process as set forth in claim 24 wherein 10 the ore treated is a feldspar.

26. A process for the froth flotation of negatively charged ores which comprises agitating and aerating an aqueous suspension of said ores in the presence of a quaternary ammonium compound having the following general formula: 15



wherein  $R_1$  represents an aliphatic hydrocarbon radical having from 12 to 18 carbon atoms, and 25  $X$  represents bromine.

SAMUEL LENHER.